

O. SCHERIEBLE.

PROCESS FOR BLEACHING AND THICKENING OILS AND FATS.  
APPLICATION FILED FEB. 14, 1913.

1,079,727.

Patented Nov. 25, 1913.

Fig. 1.



Fig. 2.



WITNESSES

John N. Horning.  
F. H. Hogan.

INVENTOR

OTTO SCHERIEBLE  
By W. H. Berrigan,  
ATTORNEY.

# UNITED STATES PATENT OFFICE.

OTTO SCHERIEBLE, OF ESSLINGEN, GERMANY.

## PROCESS FOR BLEACHING AND THICKENING OILS AND FATS.

1,079,727.

Specification of Letters Patent. Patented Nov. 25, 1913.

Application filed February 14, 1913. Serial No. 748,383.

*To all whom it may concern:*

Be it known that I, OTTO SCHERIEBLE, a citizen of the German Empire, residing at Esslingen, in the Kingdom of Wurttemburg, Germany, have invented certain new and useful Improvements in Processes for Bleaching and Thickening Oils and Fats; and I do hereby declare the following to be a full, clear, and exact description of the 10 invention, such as will enable others skilled in the art to which it appertains to make and use the same.

Large quantities of bleached and thickened pure vegetable and animal oils are constantly required industrially for the manufacture of soap and varnishes and for lubricating, as such oils have many advantages over unbleached and unthickened oil, more particularly in that the bleached and thickened oil is much more effective than ordinary oil. The supply for meeting this great demand is however somewhat limited, as the ordinary bleaching processes only supply for the market insufficient quantities of bleached oil. In the oldest process which was for a long time the only one known the oil is exposed in flat open vats or pans, for instance on roofs, to the direct action of the sun's rays, and thereby the bleaching and thickening of the oil produced. This oxidizing process however requires many weeks and only produces insufficient quantities of bleached and thickened oil, because not only is the necessary space for arranging sufficiently large containers or vats wanting, but also the process depends too much on the weather. As, however, it has now been recognized that it is more particularly the ultraviolet rays of sunlight which are actively effective in the oxidizing process, measures have recently been adopted for bleaching and thickening the oil by artificial radiation by means of electric light, the so-called uviol light, and in this way good results have been obtained. This process does not, however, meet the requirements of practical working as regards yield, and efforts are constantly being made to discover new and more profitable bleaching processes. The use of ready formed ozone in the form of ozonized air, has also not led to success in practice. However, it has now been found that by using ozone in a nascent condition, the oxidizing process is carried out very rapidly and smoothly. The process is best carried out by bringing the material to be bleached be-

tween the discharge surfaces and sending discharges directly through it, whereby the product to be bleached is maintained in violent agitation by means of the discharges (the so-called silent or brush discharges are the most effective), which pass through the oil in a continuous current, which allows of an extensive utilization of the nascent ozone produced, from oxygen, in the presence of the discharge, and by the discharge by reason of the constant rapid renewal of the absorbing surfaces. This hitherto unknown effect is the substantial feature of the present invention. The ordinary high potentials of 10,000-20,000 volts however yield no results, as oils and fats introduced between the discharge surfaces impede any discharge by reason of their great insulating properties. Various experiments in this direction have however yielded the surprising result that high potential discharges through oils and fats are quite possible when high potentials of 50,000-100,000 volts and beyond are employed. The higher therefore the potential of the electric current and the greater its frequency the more it is possible to pass a discharge with the formation of ozone through thicker layers of oil, and the greater the quantities which can be treated in the same time.

The accompanying drawing shows, by way of example, a form of apparatus by which the process may be carried out.

Figure 1 is a central vertical sectional view of the apparatus, and Fig. 2 is a perspective view of the same.

The material 5 to be bleached is placed in the pan 6, the bottom of which forms one electrode, connected to the source of electricity by the conductor 7. The second electrode 8 preferably in the form of a lattice with points 9, and fed through the conductor 10 is placed a suitable distance above the material 5 so that the discharge 11 acts upon the material 5.

The improved process is characterized by its great economy as compared with existing processes and the oils and fats made in this way have all the properties of naturally bleached and thickened products.

I declare that what I claim is:

1. A process for bleaching and thickening oils, consisting in passing a high potential current through the oil in the presence of oxygen.

2. A process for bleaching oils or fats said

- process consisting in passing an electric current of a potential of as much as 50,000 volts through the oil or fat in the presence of an atmosphere containing oxygen.
5. 3. A process of bleaching and thickening oils, consisting in passing electric discharges through the oil in the presence of oxygen.
4. A process for bleaching and thickening oils and fats, consisting in passing a silent or brush discharge through and over the oil in the presence of oxygen.
- 10 5. A process for bleaching and thickening oils and fats, consisting in passing a silent or

brush discharge through the oil in the presence of oxygen.

6. A process for bleaching and thickening oils and fats, consisting in passing a silent or brush discharge over the oil in the presence of oxygen.

In testimony whereof I affix my signature, 20  
in presence of two witnesses.

OTTO SCHERIEBLE.

Witnesses:

KARL RIETH,  
ERNEST ENTENMANN.